

1

3,469,930

## WOOL DYEING PROCESS

Patrick Harwood Harrell and Denis Ronald Lemkin, Manchester, England, assignors to Imperial Chemical Industries Limited, London, England, a corporation of Great Britain

No Drawing. Filed May 3, 1966, Ser. No. 547,157  
Claims priority, application Great Britain, May 25, 1965, 22,137

Int. Cl. D06p 1/82, 3/14

U.S. Cl. 8—54

4 Claims

### ABSTRACT OF THE DISCLOSURE

A process for dyeing wool by padding the wool in an aqueous solution of a water soluble wool dyestuff and fixing the dyestuff on the fiber by steaming wherein the padding solution contains at least 1% by weight of an alkali metal dodecylbenzene sulphonate and at least 1% by weight of a condensate of ethylene oxide with an alkyl phenol.

This invention relates to a new wool dyeing process and more particularly to a new process for dyeing wool in a continuous manner.

When wool is dyed from an aqueous dyebath, the dyestuff is quickly absorbed into the wool in an irregular manner. It has therefore long been the practice to boil the wool in the dyebath, either slightly or strongly on the acid side, this treatment serving to redistribute the dyestuff in a more even manner throughout the wool. One of the difficulties encountered in attempting to dye wool in a continuous manner is to obtain dyeings of a satisfactory levelness without subjecting the wool to a long boil in an acid bath.

It has now been found that dyeings of a satisfactory standard of levelness can be obtained on wool in a continuous dyeing process by the use of a mixture of certain surface-active agents. In accordance with the invention there is provided a process for dyeing wool by padding the wool in an aqueous solution of a water-soluble wool dyestuff and fixing the dyestuff on the fibre by steaming, wherein the padding solution contains at least 1% by weight of an alkali metal dodecylbenzene sulphonate and at least 1% by weight of a condensate of ethylene oxide with an alkyl phenol.

The alkali metal dodecyl benzene sulphonate used in the process is preferably the sodium salt; it is to be understood that by "dodecylbenzene sulphonate" there are included the commercially available materials of this name which are not pure substances but mixtures of homologues and isomers in which the main constituents are dodecylbenzene sulphonates in which the dodecyl radical can be straight chain or branched. The normal range of usage of this assistant lies between 1% and 5% by weight of the padding liquor.

The preferred condensates of ethylene oxide with an alkyl phenol are those in which from 5 to 15, and more particularly 7.5 to 10 moles of ethylene oxide, condensed with an alkyl phenol in which the alkyl radical or alkyl radicals contain from 5 to 12 carbon atoms, above all those having an octyl or nonyl radical, for example, an octyl or nonyl phenol or an octyl cresol. The normal range of usage of this assistant lies between 1% and 20% by weight of the padding liquor.

To ensure absence of alkali and hence reduce the possibility of degradation of the wool during steaming, it is preferred to add a small amount of an acid, e.g., acetic acid, to the padding liquor; as an alternative to acid there

2

can be used salts well-known as equivalents thereto in dyeing wool, for example ammonium sulphate, ammonium acetate and ammonium phosphate. A suitable quantity of acid or salt is, for example, from 0.5 to 2% by weight of the padding liquor. In addition there can be added other well-known adjuvants to dyestuff padding solutions, as used for the dyeing of other fibers, for example, thickeners such as sodium alginate and solubilizing agents, such as urea.

10 The new dyeing process can be used to apply all kinds of wool dyestuffs to the fibre; for example, anthraquinone, monoazo, 1:1-metal complex monoazo and 1:2-metal complex monoazo dyestuffs having up to 2 sulphonate acid groups, can, in general, be used. As fibres which may be dyed there may be mentioned combed slivers, also fabrics, both knitted and woven piece goods.

15 The new dyeing process can conveniently be carried out by slop-padding the wool through the dyestuff solution, removing excess of solution by passage through rollers and subjecting the wool to a steaming treatment for a period of time necessary to fix the dyestuff on the fibre, usually from 15 to 30 minutes being sufficient.

The process of the invention enables the production of strong, dyeings of an excellent standard of levelness, much superior to those obtained by the use of an alkali metal dodecyl benzene sulphonate alone or an ethylene oxide/alkyl phenol condensate alone.

20 The following examples illustrate but do not limit the invention:

### Example 1

25 Wool slubbing is passed through a solution at 20° C. containing 10 parts of the mixed 1:2-chromium complex of 1-(5'-chloro-2'-hydroxyphenylazo)-2-naphthol and 6-(4'-nitro-2'-hydroxyphenylazo)-2-acryloylamino-5-naphthol-7-sulphonic acid, 10 parts of a condensate of 9.5 moles of ethylene oxide with nonyl phenol, 10 parts of sodium dodecyl benzene sulphonate and 7.5 parts of sodium alginate per 1000 parts of liquor, and then wrung out to a liquid content of 100% on the dry weight of wool. It is then passed into a chamber heated to 100° C. with steam and steamed for 20 minutes. A level brown dyeing free from surface "frostiness" is produced.

30 If 10 parts of Carbolan Violet 2RS (Colour Index No. 62,165—C.I. Acid Violet 51) is used in place of the above dyestuff, a level violet dyeing is produced.

### Example 2

|                                           | Parts |
|-------------------------------------------|-------|
| Carbolan Violent 2RS                      | 10    |
| Alkyl/phenol condensate used in Example 1 | 40    |
| Sodium dodecyl benzene sulphonate         | 40    |
| Sodium alginate                           | 5     |
| Acetic acid                               | 5     |
| Water                                     | 900   |
|                                           | 1,000 |

60 Wool slubbing is passed at 50° C. through this solution and then through a pair of rollers to give a "pick-up" of 100% by the material followed by steaming for 15 minutes at 102° C. A level well penetrated dyeing results.

65 The 5 parts of sodium alginate can be replaced equally by 5 parts of carboxymethyl cellulose, and the 5 parts of acetic acid can be equally replaced by 20 parts of ammonium dihydrogen phosphate. In place of the alkyl/phenol condensate, there can be used the condensate of

octyl phenol with 7.5 or 8.5 moles of ethylene oxide, a similar result being obtained.

## Example 3

|                                            | Parts |
|--------------------------------------------|-------|
| Dyestuff of the formula*                   | 10    |
| Modified locust bean gum such as Indalca A | 5     |
| Ammonium dihydrogen orthophosphate         | 10    |
| Alkylphenol condensate used in Example 1   | 28    |
| Sodium dodecyl benzene sulphonate (60%)    | 18    |
| Water                                      | 929   |
|                                            | 1,000 |

\*Formula :



Wool stubbing is passed at 20° C. through this solution and then through a pair of rollers to give a liquid content of 100% on the dry weight of wool, followed by steaming for 25 minutes at 100° C. A level yellow dyeing free from surface frostiness results.

## Example 4

|                                           | Parts |
|-------------------------------------------|-------|
| Dyestuff of the formula*                  | 5     |
| Sodium alginate                           | 3     |
| Acetic acid                               | 7     |
| Alkyl phenol condensate used in Example 1 | 16    |
| Sodium dodecyl benzene sulphonate (60%)   | 10    |
| Water                                     | 959   |
|                                           | 1,000 |

\*Formula :



Pad wool stubbing at 20° C. to 100% pick-up, steam for 15 minutes at 102° C. A level blue dyeing is produced.

## Example 5

|                                          | Parts |
|------------------------------------------|-------|
| Dyestuff of the formula*                 | 15    |
| Sodium alginate                          | 5     |
| Acetic acid                              | 8     |
| Alkylphenol condensate used in Example 1 | 40    |
| Sodium dodecyl benzene sulphonate (60%)  | 26    |
| Water                                    | 906   |
|                                          | 1,000 |

\*Formula :

(Copper phthalocyanine)  $(3-\text{SO}_3\text{H})_{1,2}$   $(3-\text{SO}_2\text{NHCH}_2\text{CH}_2\text{Cl})_{1,5}$   $(3-\text{SO}_2\text{NH}_2)_{1,6}$  70

Worsted serge is passed at 30° C. through the solution, squeezed to 100% expression and steamed for 25 minutes at 102° C. A level, well-penetrated blue dyeing is produced.

## Example 6

|                                                                                                                                                                                      | Parts |
|--------------------------------------------------------------------------------------------------------------------------------------------------------------------------------------|-------|
| Mixed 1:2-chromium complex of 4-nitro-2-amino-phenol $\rightarrow$ 1-phenyl-3-methyl-5-pyrazolone and 4-nitro-2-aminophenol $\rightarrow$ 2-acetylaminoo-8-naphthol-6-sulphonic acid | 5     |
| Modified locust bean gum                                                                                                                                                             | 5     |
| Ammonium sulphate                                                                                                                                                                    | 10    |
| Alkylphenol condensate used in Example 1                                                                                                                                             | 16    |
| Sodium dodecyl benzene sulphonate (60%)                                                                                                                                              | 10    |
| Water                                                                                                                                                                                | 954   |
|                                                                                                                                                                                      | 1,000 |

1,000

Wool stubbing is padded through this solution at 50° C. and squeezed to give 100% pick-up and is then steamed for 15 minutes at 100° C. A level brown dyeing results.

## Example 7

|                                                  | Parts |
|--------------------------------------------------|-------|
| 1:2-chromium complex of the dyestuff of formula* | 15    |
| Sodium alginate                                  | 5     |
| Ammonium dihydrogen phosphate                    | 15    |
| Alkylphenol condensate used in Example 1         | 40    |
| Sodium dodecyl benzene sulphonate                | 16    |
| Water                                            | 909   |
|                                                  | 1,000 |

\*Formula :



Wool stubbing is padded through this solution at 20° C., squeezed to give 100% pick-up and is then steamed for 25 minutes at 102° C. A level brown dyeing free from surface frostiness results.

## Example 8

|                                          | Parts |
|------------------------------------------|-------|
| Dyestuff of the formula*                 | 40    |
| Modified locust bean gum                 | 5     |
| Alkylphenol condensate used in Example 1 | 40    |
| Sodium dodecyl benzene sulphonate        | 16    |
| Chromium fluoride                        | 50    |
| Acetic acid                              | 10    |
| Water                                    | 839   |
|                                          | 1,000 |

\*Formula :



Wool stubbing is padded in this solution to 100% expression and steamed for 30 minutes at 102° C. A level black dyeing is produced.

5

The 10 parts of acetic acid may be replaced equally well by 20 parts of oxalic acid.

We claim:

1. A process for dyeing wool by padding the wool in an aqueous acidic solution of a water-soluble wool dyestuff and fixing the dyestuff on the fibre by steaming, wherein the padding solution contains at least 1% by weight of an alkali metal dodecylbenzene sulphonate and at least 1% by weight of a condensate of ethylene oxide with an alkyl phenol wherein there are from 5 to 15 moles of ethylene oxide per mole of alkyl phenol.

2. A process as claimed in claim 1 wherein the alkyl phenol has 5 to 12 carbon atoms in the alkyl moiety.

3. A process as claimed in claim 2 wherein there is used a condensate of from 7.5 to 10 moles of ethylene oxide with a phenol selected from the group consisting of octyl phenol and nonyl phenol.

5

10

6

4. A process as claimed in claim 1 in which an acidic material selected from the group consisting of acetic acid, ammonium sulphate, ammonium acetate and ammonium phosphate is added to the padding solution.

## References Cited

UNITED STATES PATENTS

3,377,130 4/1968 Millson et al.

3,391,985 7/1968 Furbuchen et al.

NORMAN G. TORCHIN, Primary Examiner

J. E. CALLAGHAN, Assistant Examiner

U.S. Cl. X.R.

8—90, 92